# EUROPEAN PATENT SPECIFICATION

(11) **EP 1 846 610 B1**
(45) Date of publication and mention of the grant of the patent: **01.09.2010**
(21) Application number: 05823829.6
(22) Date of filing: 21.12.2005
(51) Int. Cl.: D06M 13/272, D06P 1/62, D06P 3/52, D06M 101/32

(54) **DISPERSANT FOR POLYESTER OLIGOMERS**
DISPERGIERMITTEL FÜR POLYESTEROLIGOMERE
AGENT DISPERSANT POUR DES OLIGOMERES POLYESTERS

(30) Priority: 23.12.2004 EP 04030576
(43) Date of publication of application: 24.10.2007
(73) Proprietor: Clariant Finance (BVI) Limited, Road Town, Tortola (VG)
(72) Inventor: JUNGEN, Manfred House No.212, Shanghai 201702 (HK)
(74) Representative: Jacobi, Carola
(86) International application number: PCT/EP2005/057062
(87) International publication number: WO 2006/067199

(56) References cited:
- WO-A-2004/090222
- DE-A1- 19 516 957

## Description

The present invention relates to the use of alpha-olefinsulphonates as a dispersant for polyester oligomers.

Polyester fibres are produced by a process which gives rise, not only in the fibre material but also on the fibre surface, to cyclic or linear oligomers which can lead to various problems in the course of the later processing of the fibres. Especially the cyclic trimers of polyethylene terephthalate present difficulties. These oligomers are not dyeable and possess only minimal solubility in water. They therefore crystallize on contact with the aqueous dyeing liquor and cause troublesome deposits on the surface of the fibre and in dyeing machines. As well as to possible unlevelness of the dyeing, these deposits can lead to soiling, dust and damage of sensitive parts in the course of the further processing.

Hodul et al. review the matter in Vlákna a textil 5(1-2), 12-18, 1998. It was found that sodium laurylsulphate shows some effect as a dispersant.

WO 2004/090222 A2 describes a textile auxiliary based on 2-acrylamido-2-methylpropanesulphonic acid (AMPS) and a polymer based on acrylic acid and/or maleic acid as an oligomer dispersant.

In the textile industry, however, there continues to be a demand for suitable ways to eliminate these oligomers. It has now been found that, surprisingly, certain alpha-olefinsulphonates, which may be poly- as well as monounsaturated, constitute excellent dispersants for polyester oligomers, either alone or in combination with further codispersants. This surprising dispersing effect removes the undesirable oligomers from the fibre or the textile fabric, but also from the textile-dyeing machines, so that these are very simple and efficient to clean, or prevents the production of deposits in the first place. This good dispersing effect can also be utilized for deweighting.

The present invention accordingly provides for the use of mono- or polyunsaturated alpha-olefinsulphonates as an active substance alone or in combination with further codispersants for removing polyester oligomers from fibres, fabrics or textile-dyeing machines, for preventing deposits or for deweighting polyester fibres.

The alpha-olefinsulphonates are substances of the general formula (I)

R-CH=CH-CH₂-SO₃-M (I)

where
- R: is a linear or branched alkyl radical or a linear or branched, mono- or polyunsaturated alkenyl radical having 7 to 23 carbon atoms, and
- M: is hydrogen, an alkali metal, ammonium or substituted ammonium.

Preference is given to substances wherein
- R: is a linear alkyl radical or alkenyl radical having 11 to 15 carbon atoms, and
- M: is sodium or ammonium.

Particular preference is given to substances wherein
- R: is a linear alkyl radical having 11 to 15 carbon atoms, and
- M: is sodium.

Useful further codispersants include the following compounds: aryl or alkyl sulphonates and sulphates, for example cumenesulphonate, aromatic esters and amides, for example N-substituted phthalimides, benzyl benzoate and further benzoic esters, mono- or oligoesters of terephthalic acid with a polyol, ditto for phthalic acid and isophthalic acid, aryl alkoxylates, aryl-formaldehyde condensates sulphated and non-sulphated, phosphates and phosphonates of the aforementioned compounds, sulphated, sulphonated, phosphated, phosphonated olefin derivatives, for example oleyl alcohols or oleic acid derivatives.

The alpha-olefinsulphonates mentioned are known substances and are preparable by known methods.

The active substance can be used directly as such or else in aqueous mixture, in which case the aqueous mixture utilizes 10% to 40% by weight of active substance with or without up to 4% by weight of further additives.

Preferably, the aqueous mixture comprises 20% to 30% by weight of active substance and also, if appropriate, up to 2% by weight each of sodium cumenesulphonate, free oleic acid, sulphated oleic acid or other dispersing agents that are customary in the textile industry and known to one skilled in the art, or other auxiliary materials. A methylated phenol ethoxylate-formaldehyde condensate is used as a preferred further dispersing agent.

It may also be helpful in some instances for a compound of the formula (II)

R-C(OH)H-CH₂-CH₂-SO₃-M (II)

where
- R: is a linear or branched alkyl radical having 7 to 23 carbon atoms, and
- M: is hydrogen, an alkali metal, ammonium or substituted ammonium,
to be used as a further active substance, in which case the amount of (II) is in the range from 1% to 10% by weight of the amount of (I).

Preferably, in the formula (II),
- R: is a linear alkyl radical having 11 to 15 carbon atoms,
- M: is sodium, and
the amount of (II) is in the range from 1% to 5% by weight of the amount of (I).

The aqueous mixture can be added to the dyebath directly in a concentration of 0.5 to 4 ml/l and preferably in a concentration of 1 to 3 ml/l. Existing processes may be employed, for example the exhaust process, using a jigger, a winch beck or a jet-dyeing machine for woven and knitted material or in a dyeing apparatus for polyester yarn and also polyester staple. Customary further dyeing auxiliaries can be used alongside the dispersant of the present invention.

Since the deposition of polyester oligomers in textile-dyeing machines can lead to various problems, the surprisingly good dispersing effect described above constitutes a substantial technical benefit, since the active substance or its aqueous mixtures can thus also be used for cleaning the textile-dyeing machines. The machines can be treated under neutral, acidic or basic conditions, preferably they are boiled out in the additional presence of caustic soda and sodium hydrosulphite (or yet further auxiliary surfactants), which leads to complete removal of the polyester oligomers. But the use according to the present invention can also prevent the formation of deposits in the first place.

Furthermore, the alpha-olefinsulphonates described or their aqueous mixtures, if appropriate in the identified combination with a further active substance or further codispersants, can be used for deweighting. Deweighting is an alkaline pretreatment of the surface of polyester fibres whereby a controllable peeling effect is achieved, which leads to a silky, soft hand.

The examples which follow illustrate the invention.

### TEST METHOD

The test method described in WO 2004/090222 appeared to be somewhat removed from actual commercial practice, which is why direct large-scale trials under industrial conditions were carried out. In each trial, about 50 kg of polyester yarn were exhaust dyed with various disperse dyes (liquor ratio 11.3:1; pH 4.5-5.5; bath temperature 80-135°C, reduction clearing with NaOH/sodium dithionite, neutralization with acetic acid).

A dispersant based on lauryl ether sulphate/aryl sulphonate was used as a comparison against the prior art.

### RESULTS OF PRACTICAL TRIALS

The comparative product showed distinct deposits on the surface of the dyed packages, whereas this was not the case with the dispersant of the present invention. This was particularly noticeable in the case of yarn packages dyed black. Figure 1 shows distinct deposits on using the comparative dispersant. Figure 2 shows that there are no deposits to be seen on the package surface when the dispersant of the present invention is used, all one can see is a uniformly black surface.

It was also determined that the dispersant of the present invention has no adverse effect on the light-fastness of polyester dyeings or on the dyed result (hue, bath exhaustion, for example).

## Claims

1. Use of mono- or polyunsaturated alpha-olefinsulphonates as an active substance alone or in combination with further codispersants for removing polyester oligomers from fibres, fabrics or textile-dyeing machines, for preventing deposits or for deweighting polyester fibres.

2. Use according to Claim 1, **characterized in that** the alpha-olefinsulphonates are substances of the general formula (I)
R-CH=CH-CH₂-SO₃-M (I)
where
R is a linear or branched alkyl radical or a linear or branched, mono- or polyunsaturated alkenyl radical having 7 to 23 carbon atoms, and
M is hydrogen, an alkali metal, ammonium or substituted ammonium.

3. Use according to Claim 2, wherein
R is a linear alkyl radical or alkenyl radical having 11 to 15 carbon atoms, and
M is sodium or ammonium.

4. Use according to Claim 3, wherein
R is a linear alkyl radical having 11 to 15 carbon atoms, and
M is sodium.

5. Use according to at least one of the preceding claims, **characterized in that** aryl or alkyl sulphonates and sulphates, aromatic esters and amides, aryl alkoxylates, aryl-formaldehyde condensates sulphated and non-sulphated, phosphates and phosphonates of the aforementioned compounds and also sulphated, sulphonated, phosphated or phosphonated olefin derivatives are used as further codispersants.

6. Use according to at least one of the preceding claims, **characterized in that** the active substance is used alone or **in that** 10% to 40% by weight of active substance is used in an aqueous mixture together with 0% to 4% by weight of further additives.

7. Use according to Claim 6, **characterized in that** the aqueous mixture comprises 20% to 30% by weight of active substance and also 0% to 2% by weight each of sodium cumenesulphonate, free oleic acid, sulphated oleic acid or other dispersing agents.

8. Use according to at least one of the preceding claims, **characterized in that** a compound of the formula (II)
R-C(OH)H-CH₂-CH₂-SO₃-M (II)
where
R is a linear or branched alkyl radical having 7 to 23 carbon atoms, and
M is hydrogen, an alkali metal, ammonium or substituted ammonium,
is used as a further active substance, the amount of (II) being in the range from 1% to 10% by weight of the amount of (I).

9. Use according to Claim 8, wherein
R is a linear alkyl radical having 11 to 15 carbon atoms, and
M is sodium, and wherein
the amount of (II) is in the range from 1% to 5% by weight of the amount of (I).

10. Use according to at least one of the preceding claims, **characterized in that** the textile-dyeing machines are treated with active substance or aqueous mixtures thereof under neutral, acidic or alkali conditions, preferably in the presence of caustic soda and of sodium hydrosulphite and also in the presence or absence of further auxiliary surfactants.

11. Use of an aqueous mixture of Claim 6 or 7 for removing polyester oligomers from fibres, fabrics or textile-dyeing machines or for preventing deposits in a process for dyeing polyester fibres or material, which comprises adding 0.5 to 4 ml/l to the dyeing liquor.

12. Use according to Claim 11, wherein the dyeing is carried out in an exhaust process, the liquor ratio is in the range from 3:1 to 20:1, preferably in the range from 5:1 to 13:1 and more preferably in the range from 6:1 to 11:1, the pH is in the range from 3 to 7 and preferably in the range from 4 to 5.5, and the dyeing temperature is between 50 and 150°C, preferably between 95 and 140°C and more preferably between 110 and 135°C.

13. Use according to Claim 11, wherein the dyeing is carried out a pH in the range from 7 to 11 and preferably in the range from 8 to 10.

## Patentansprüche

1. Verwendung von einfach oder mehrfach ungesättigten alpha-Olefinsulfonaten als Aktivsubstanz alleine oder in Kombination mit weiteren Codispergatoren zum Entfernen von Polyesteroligomeren aus Fasern, Textilgeweben oder Textilfärbemaschinen, zum Verhindern von Ablagerungen oder für das "deweighting" von Polyesterfasern.

2. Verwendung gemäss Anspruch 1, **dadurch gekennzeichnet, dass** es sich bei den alpha-Olefinsulfonaten um Substanzen der allgemeinen Formel (I)
R-CH=CH-CH₂-SO₃-M (I)
handelt, wobei
R einen linearen oder verzweigten Alkylrest oder einen linearen oder verzweigten, einfach oder mehrfach ungesättigten Alkenylrest mit 7 bis 23 Kohlenstoffatomen und
M Wasserstoff, ein Alkalimetall, Ammonium oder substituiertes Ammonium bedeutet.

3. Verwendung gemäss Anspruch 2, wobei
R einen linearen Alkylrest oder Alkenylrest mit 11 bis 15 Kohlenstoffatomen und
M Natrium oder Ammonium bedeutet.

4. Verwendung gemäss Anspruch 3, wobei
R einen linearen Alkylrest mit 11 bis 15 Kohlenstoffatomen und
M Natrium bedeutet.

5. Verwendung gemäss mindestens einem der vorangehenden Ansprüche, **dadurch gekennzeichnet, dass** als weitere Codispergatoren Aryl- oder Alkylsulfonate und -sulfate, aromatische Ester und Amide, Arylalkoxylate, Aryl-Formaldehydkondensate sulfatiert und nicht sulfatiert, Phosphate und Phosphonate der vorab genannten Verbindungen, sowie sulfatierte, sulfonierte, phosphatierte oder phosphonierte Olefinderivate eingesetzt werden.

6. Verwendung gemäss mindestens einem der vorangehenden Ansprüche, **dadurch gekennzeichnet, dass** die Aktivsubstanz allein oder dass 10 bis 40 Gew.-% Aktivsubstanz in einer wässrigen Mischung zusammen mit 0 bis 4 Gew.-% weiterer Additive verwendet wird.

7. Verwendung gemäss Anspruch 6, **dadurch gekennzeichnet, dass** die wässrige Mischung 20 bis 30 Gew.-% Aktivsubstanz sowie jeweils 0 bis 2 Gew.-% Natriumcumolsulfonat, freie Ölsäure, sulfatierte Ölsäure oder andere Dispergiermittel enthält.

8. Verwendung gemäss mindestens einem der vorangehenden Ansprüche, **dadurch gekennzeichnet, dass** als weitere Aktivsubstanz eine Verbindung der Formel (II)
R-C(OH)H-CH₂-CH₂-SO₃-M (II)
wobei
R einen linearen oder verzweigten Alkylrest mit 7 bis 23 Kohlenstoffatomen und
M Wasserstoff, ein Alkalimetall, Ammonium oder substituiertes Ammonium bedeutet, eingesetzt wird, wobei die Menge an (II) 1 bis 10 Gew.-% der Menge an (I) beträgt.

9. Verwendung gemäss Anspruch 8, wobei
R einen linearen Alkylrest mit 11 bis 15 Kohlenstoffatomen und
M Natrium bedeutet, und wobei
die Menge an (II) 1 bis 5 Gew.-% der Menge an (I) beträgt.

10. Verwendung gemäss mindestens einem der vorhergehenden Ansprüche, **dadurch gekennzeichnet, dass** die Textilfärbemaschinen unter neutralen, sauren oder alkalischen Bedingungen, vorzugsweise unter Zugabe von Natronlauge und von Na-Hydrosulfit sowie gegegebenenfalls von weiteren Hilfstensiden, mit Aktivsubstanz oder wässrigen Mischungen davon behandelt werden.

11. Verwendung einer wässrigen Mischung gemäss den Ansprüchen 6 oder 7 zum Entfernen von Polyesteroligomeren aus Fasern, Textilgeweben oder Textilfärbemaschinen oder zum Verhindern von Ablagerungen in einem Verfahren zum Färben von Polyesterfasern oder -material, wobei 0,5 bis 4 ml/l zur Färbeflotte zugegeben werden.

12. Verwendung gemäss Anspruch 11, wobei die Färbung im Ausziehverfahren erfolgt, das Flottenverhältnis 1:3 bis 1:20, vorzugsweise 1:5 bis 1:13, besonders bevorzugt 1:6 bis 1:11 und der pH-Wert 3 bis 7, vorzugsweise 4 bis 5,5 beträgt, und die Färbetemperatur zwischen 50 und 150°C, vorzugsweise zwischen 95 und 140°C, besonders bevorzugt zwischen 110 und 135°C liegt.

13. Verwendung gemäss Anspruch 11, wobei bei einem pH von 7 bis 11, vorzugsweise von 8 bis 10, gefärbt wird.

## Revendications

1. Utilisation d'alpha-oléfinesulfonates mono- ou poly-insaturés en tant que substance active seuls ou en combinaison avec des codispersants supplémentaires pour éliminer les oligomères de polyester de machines de coloration de fibres, tissus ou textiles, pour prévenir les dépôts ou pour décharger des fibres de polyester.

2. Utilisation selon la revendication 1, **caractérisée en ce que** les alpha-oléfinesulfonates sont des substances de formule générale (I)
R-CH=CH-CH₂-SO₃-M (I)
où
R est un radical alkyle linéaire ou ramifié ou un radical alcényle linéaire ou ramifié, mono- ou poly-insaturé ayant de 7 à 23 atomes de carbone, et
M est un hydrogène, un métal alcalin, un ammonium ou un ammonium substitué.

3. Utilisation selon la revendication 2, dans laquelle
R est un radical alkyle ou un radical alcényle linéaire ayant de 11 à 15 atomes de carbone, et
M est un sodium ou un ammonium.

4. Utilisation selon la revendication 3, dans laquelle
R est un radical alkyle linéaire ayant de 11 à 15 atomes de carbone, et
M est un sodium.

5. Utilisation selon au moins une des revendications précédentes, **caractérisée en ce que** des aryl- ou alkylsulfonates et sulfates, des esters et amides aromatiques, des alcoxylates d'aryle, des condensats aryl-formaldéhyde sulfatés et non sulfatés, des phosphates et des phosphonates des composés mentionnés ci-dessus et également des dérivés d'oléfine sulfatés, sulfonés, phosphatés ou phosphonatés sont utilisés en tant que codispersants supplémentaires.

6. Utilisation selon au moins une des revendications précédentes, **caractérisée en ce que** la substance active est utilisée seule ou **en ce que** 10 % à 40 % en poids de substance active sont utilisés en mélange aqueux conjointement avec 0 % à 4 % en poids d'additifs supplémentaires.

7. Utilisation selon la revendication 6, **caractérisée en ce que** le mélange aqueux comprend de 20 % à 30 % en poids de substance active et également de 0 % à 2 % en poids chacun de cumènesulfonate de sodium, d'acide oléique libre, d'acide oléique sulfaté ou d'autres agents dispersants.

8. Utilisation selon au moins une des revendications précédentes, **caractérisée en ce qu'**un composé de formule (II)
R-C (OH) H-CH₂-CH₂-SO₃-M (II)
où
R est un radical alkyle linéaire ou ramifié ayant de 7 à 23 atomes de carbone, et
M est un hydrogène, un métal alcalin, un ammonium ou un ammonium substitué,
est utilisé en tant que substance active supplémentaire, la quantité de (II) étant dans la plage de 1 % à 10 % en poids de la quantité de (I).

9. Utilisation selon la revendication 8, dans laquelle
R est un radical alkyle linéaire ayant de 11 à 15 atomes de carbone, et
M est un sodium, où
la quantité de (II) est dans la plage de 1 % à 5 % en poids de la quantité de (I).

10. Utilisation selon au moins une des revendications précédentes, **caractérisée en ce que** les machines de coloration de textile sont traitées avec une substance active ou des mélanges aqueux de celles-ci dans des conditions neutres, acides ou alcalines, de préférence en présence de soude caustique et d'hydrosulfite de sodium et également en présence ou en l'absence de tensioactifs auxiliaires supplémentaires.

11. Utilisation d'un mélange aqueux de la revendication 6 ou 7 pour éliminer des oligomères de polyester de machines de coloration de fibres, tissus ou textiles ou pour prévenir les dépôts dans un procédé de coloration de fibres ou matériau de polyester, qui comprend l'ajout de 0,5 à 4 ml/l à la liqueur de coloration.

12. Utilisation selon la revendication 11, dans laquelle la coloration est effectuée dans un procédé d'épuisement, le rapport de liqueur est dans la plage de 3:1 à 20:1, de préférence dans la plage de 5:1 à 13:1 et plus préférablement dans la plage de 6:1 à 11:1, le pH est dans la plage de 3 à 7 et de préférence dans la plage de 4 à 5,5, et la température de coloration est comprise entre 50 et 150 °C, de préférence entre 95 et 140 °C et plus préférablement entre 110 et 135 °C.

13. Utilisation selon la revendication 11, dans laquelle la coloration est effectuée à un pH dans la plage de 7 à 11 et de préférence dans la plage de 8 à 10.
